

UNITED STATES PATENT OFFICE

**2,438,452**

## **DIESEL ENGINE FUELS**

**Robert T. Pollock, New York, N. Y.**

**No Drawing. Application January 20, 1945,  
Serial No. 573,812**

**2 Claims. (Cl. 44—57)**

1

This invention relates to internal combustion engine fuels and relates more particularly to fuels for compression ignition engines and to methods and means for improving their ignition qualities.

Objects and advantages of the invention will be set forth in part hereinafter and in part will be obvious herefrom, or may be learned by practice with the invention, the same being realized and attained by means of the steps, compositions, combinations and improvements pointed out in the appended claims.

The invention consists in the novel steps, compositions, combinations and improvements herein described.

Objects of this invention are to make possible the raising of the cetane number of fuels for compression ignition engines without lowering, or without substantial lowering of the flash point of the fuel and with some lowering of the pour point of the fuel; and, to accomplish the foregoing through the use of an addition agent or additive material which is stable and will not decompose under normal storage conditions, which is non-toxic and non-explosive and is non-inflammable at room temperature and which is liquid even at very low temperatures such, for example, as -60° F. and which does not increase the amount of precipitant, if any, of a fuel to which it may be added, nor adversely affect the normal color of the fuel upon addition or after prolonged storage.

The invention comprises the method and means as more fully set forth hereinafter.

By way of introduction, it is to be understood that alkyl carbamates are the urethanes,

$$\text{NH}_2\text{CO}_2\text{R}$$

wherein R is an alkyl group. Where R above is the ethyl group,  $C_2H_5$ , the resulting ethyl carbamate,  $NH_2CO_2Et$ , is commonly termed urethane. However, where R above is an alkyl group other than the ethyl group, e. g., methyl, propyl, butyl, etc., it is customary to identify the alkyl carbamate by reference to the particular alkyl group employed. Thus, the alkyl carbamate,  $NH_2CO_2CH_3$ , is termed methyl carbamate; the

2

alkyl carbamate,  $\text{NH}_2\text{CO}_2\text{C}_3\text{H}_7$ , is termed propyl carbamate; the alkyl carbamate,  $\text{NH}_2\text{CO}_2\text{C}_4\text{H}_9$ , is termed butyl carbamate, and so on.

To the accomplishment of the foregoing ends and objects and in accordance with this invention, there is incorporated in a hydrocarbon oil constituting the fuel whose cetane rating is to be raised a small quantity of an addition agent, having the formula:



wherein R and R' are alkyl radicals which may be the same or different and of which N-nitro N-butyl urethan; N-nitro N-isopropyl urethan; N-nitro N-ethyl urethan; N-nitro N-methyl urethan and N-nitro N-butyl, butyl carbamate, are typical.

The incorporation is preferably effected by mixing the addition agent directly with the fuel which may then be fed to the combustion zone of the engine in the usual manner. Alternatively, the agent may be introduced with the intake air in small amounts separate from the main fuel spray or may be injected a few degrees ahead of the main spray.

30 The quantity of the agent to be added is advantageously in the order of one percent (1%) by weight of the fuel treated, although a greater or less quantity may be employed to effect a greater or less change in the cetane number of the fuel as may be desired.

As may be seen by reference to the following table of comparative data of a typical Diesel engine fuel in a treated and untreated state, the presence of a small quantity of the addition agent results in the treated fuel having a materially higher cetane number than the neat fuel. This increase in the cetane number is accomplished without reduction in the flash point of the fuel, or at most with a relatively minor lowering of the flash point. A corollary advantage, moreover, resides in the fact that the pour point

of the fuel is lowered thus improving the utility of the fuel for general industrial and military purposes.

|                                | Col. I<br>Neat Fuel | Col. II<br>Neat Fuel +<br>1% Add. | Col. III<br>Neat Fuel +<br>2% Add. |
|--------------------------------|---------------------|-----------------------------------|------------------------------------|
| Flash Point (P. M.)            | 203° F.             | 203° F.                           | 203° F.                            |
| Pour Point                     | -12° F.             | -16° F.                           | -21° F.                            |
| Viscosity (Saybolt) at 100° F. | 35.2 secs.          | 35.6 secs.                        | 35.4 secs.                         |
| Water and Sediment             | nill                | nill                              | nill                               |
| Sulfur                         | 0.22%               | 0.22%                             | 0.21%                              |
| Carbon Residue                 | 0.01%               | 0.03%                             | 0.08%                              |
| Carbon Residue on 10% Bottoms  | 0.21%               | 0.52%                             | 1.09%                              |
| Ash                            | nill                | nill                              | nill                               |
| Corrosion at 212° F.           | Passes              | Passes                            | Passes                             |
| 90% Distillation Pt.           | 552° F.             | 593° F.                           | 584° F.                            |
| Color (N. P. A.)               | 4.5                 | 4.5                               | 4.5                                |
| Cetane Number                  | 39                  | 50                                | 55                                 |
| Diesel Index                   | 42.4                | 41.7                              | 40.8                               |
| Aniline Point                  | 132.8° F.           | 122.5° F.                         | 131.9° F.                          |
| Gravity                        | 31.9                | 31.4                              | 30.9                               |
| Temperature Distillation:      |                     |                                   |                                    |
| IB Pt.                         | 420° F.             | 435° F.                           | 426° F.                            |
| 5% off.                        | 448° F.             | 457° F.                           | 454° F.                            |
| 10                             | 455° F.             | 465° F.                           | 464° F.                            |
| 20                             | 470° F.             | 477° F.                           | 478° F.                            |
| 30                             | 482° F.             | 485° F.                           | 487° F.                            |
| 40                             | 493° F.             | 496° F.                           | 496° F.                            |
| 50                             | 503° F.             | 506° F.                           | 508° F.                            |
| 60                             | 517° F.             | 517° F.                           | 521° F.                            |
| 70                             | 532° F.             | 532° F.                           | 532° F.                            |
| 80                             | 551° F.             | 550° F.                           | 554° F.                            |
| 90                             | 582° F.             | 583° F.                           | 584° F.                            |
| 95                             | 608° F.             | 618° F.                           | 610° F.                            |
| E Pt.                          | 640° F.             | 625-98%                           | 640-98.5%                          |

In the foregoing table the addition agent employed is N-nitro N-butyl urethan and it will be observed that the addition of 1% wt. of this compound (col. II) raised the cetane number of the neat fuel (col. I) from 39 to the generally recognised permissible minimum of 50. A further addition of 1% (col. III) raised the cetane number still further to above the permissible minimum, without degradation of the flash point and with a further beneficial lowering of the pour point.

Other members of the class having the general formula above mentioned exhibit the same general beneficial properties with variations in minor degree and are equally suitable for the purpose. 45

The invention in its broader aspects is not limited to the specific steps, compositions, combinations and improvements described but departures may be made therefrom within the scope of the accompanying claims without departing from the principles of the invention and without sacrificing its chief advantages.

What I claim is:

1. A fuel for compression ignition engines comprising a hydrocarbon Diesel oil containing a small quantity, at least sufficient to increase the cetane rating of said oil, of a material having the formula



wherein R and R' are alkyl radicals.

2. A fuel for compression ignition engines comprising a hydrocarbon Diesel oil containing about 1% by weight of a material having the formula



wherein R and R' are alkyl radicals.

30 ROBERT T. POLLOCK.

#### REFERENCES CITED

The following references are of record in the file of this patent:

#### UNITED STATES PATENTS

| Number    | Name  | Date          |
|-----------|-------|---------------|
| 2,274,629 | Ellis | Feb. 24, 1942 |
| 2,274,665 | Clark | Mar. 3, 1942  |

#### FOREIGN PATENTS

| Number  | Country       | Date         |
|---------|---------------|--------------|
| 405,658 | Great Britain | Feb. 5, 1934 |